

1,202,887.

W. J. PHELPS,

SASH WEIGHT.

APPLICATION FILED NOV. 24, 1914.

Patented Oct. 31, 1916.

Fig. 1.



Fig. 4.



WITNESSES

Howard D. Orr.  
F. T. Chapman.

Fig. 2.



Fig. 3.



Walter J. Phelps, INVENTOR,

BY *E. G. Siggers*

ATTORNEY

# UNITED STATES PATENT OFFICE.

WALTER J. PHELPS, OF BALTIMORE, MARYLAND, ASSIGNOR TO THE PHELPS COMPANY, OF WEIRTON, WEST VIRGINIA, A CORPORATION OF WEST VIRGINIA.

## SASH-WEIGHT.

1,202,887.

Specification of Letters Patent.

Patented Oct. 31, 1916.

Application filed November 24, 1914. Serial No. 873,804.

*To all whom it may concern:*

Be it known that I, WALTER J. PHELPS, a citizen of the United States, residing in Baltimore and State of Maryland, have invented a new and useful Sash-Weight, of which the following is a specification.

This invention has reference to sash weights, especially of the kind employing lead as the body material, and its object is 10 to provide a sash weight having characteristics of an all-lead sash weight with certain objectionable features eliminated, and possessing additional advantages.

Among the disadvantages of all-lead sash 15 weights are the relatively high cost of lead and the liability of bending and denting the sash weights due to the softness of the metal employed. Among the advantages of lead sash weights are the relatively small bulk 20 for a given weight and the smooth exterior whereby lead sash weights have and are replacing iron sash weights in the better class of buildings, since iron sash weights are brittle and of a rough exterior due to the 25 material from which they are customarily manufactured.

In accordance with the present invention lead is utilized as in the all-lead sash weights, but there is also utilized a material 30 heretofore largely employed in the production of sash weights and with which lead readily unites. This last-named material is a waste product of factories producing tin articles from sheet tin or tin plate, and 35 which is customarily known as tin scrap. The tin scrap is treated with molten lead by means of which either of two conditions are brought about. The molten lead alloys with the tin and becomes as tenaciously adherent 40 to the steel base of the tin plate as characterized the tenacious clinging of the tin to the base. The molten lead by its alloying action with the tin greatly dilutes the tin and a large proportion of the tin may be re- 45 covered from the mass in the form of an alloy of lead and tin with the lead greatly predominating. Or, the tin values need not be recovered at all. In either case the sash weights are formed of a mixture of lead 50 and tin scraps with an alloy of tin and lead in tenacious adherence to the basic material of the tin scraps and either all the tin originally contained in the tin scraps, or but a

fractional proportion thereof is contained in the mixture.

The relative weights of the materials employed are such that a sash weight composed in most part of tin scraps with the remainder formed of lead united to the tin scraps while the lead is molten is of somewhat 55 greater bulk than an all lead sash weight, but of materially less bulk than an iron sash weight. From exterior appearance the composite sash weight of the present invention is practically identical with an all lead sash 60 weight, but because of the presence of the relatively very cheap tin scrap the cost of production of the sash weight is far less 65 than that of an all lead sash weight.

The invention will be best understood 70 from a consideration of the following detailed description, taken in connection with the accompanying drawings forming a part of this specification, with the further understanding that while the drawings show a 75 practical form of the invention, the latter is not confined to any strict conformity with the showing of the drawings, but may be changed and modified so long as such changes and modifications mark no material 80 departure from the salient features of the invention.

In the drawings, Figure 1 is a perspective view of a sash weight constructed in accordance with the present invention and more or 85 less schematically representing some features of the invention. Fig. 2 is an enlarged schematic view of a minute fragment of a sash weight constructed in accordance with the present invention. Fig. 3 is a cross-section of the sash weight of Fig. 1 on an enlarged scale and more or less schematically 90 illustrating certain features thereof. Fig. 4 is an elevation with parts in section of a composite sash weight embodying the present 95 invention.

Referring to the drawings there is shown in Fig. 1 a sash weight 1 which may follow any of the usual conformations of such articles, and may also be taken as representative 100 of any article other than a sash weight to which the material of the present invention is adapted. The sash weight 1 has a body portion of lead infiltrated throughout or substantially throughout with small pieces 105 2 of tin plate either with the tin coating re-

maining thereon or removed therefrom entirely or to a greater or less extent.

In the practical embodiment of the invention the tin scrap may represent from 5 fifty to seventy-five per cent. more or less of either the weight or the bulk of the completed article.

The facility with which lead will alloy with tin is of material advantage in the 10 present invention, since because of this characteristic the tin scrap or the steel base thereof becomes so tenaciously united with the lead mass that the resultant article is in effect a one piece structure where all the 15 parts, though of individually different characteristics, are, so far as their union is concerned, practically homogeneous.

In Fig. 2 the attempt is made to more or less schematically represent the conditions 20 occurring when the tin scrap and molten lead are brought together.

At 2<sup>a</sup> in Fig. 2 is represented a minute fragment on a greatly enlarged scale of a piece of sheet steel constituting the base of 25 tin plate. This sheet of steel is covered on opposite faces with a thin coating 2<sup>b</sup> of tin very tenaciously united to the steel in the course of manufacture, so that the union approaches that which would occur if the 30 coating 2<sup>b</sup> were integral with the base 2<sup>a</sup>.

When molten lead is applied to the tinned sheet, which lead is indicated at 2<sup>c</sup> in Fig. 2, the lead alloys with the tin, and this is indicated in Fig. 2 by an intermixture of 35 the section lines of the lead mass 2<sup>c</sup> and the tin coating 2<sup>b</sup>. This alloying action may proceed so far as to rob the steel sheet of all the original tin coating which is replaced by a coating of lead and tin very 40 weak in tin because of the distribution of the latter through the lead, but such substitute coating is in as firm and tenacious union with the steel as was the original tin coating.

45 Under present commercial conditions tin scrap is of relatively small value and the manufacturer of articles made of tin plate can dispose of the waste tin in the form of tin scrap only at a price far below the cost 50 to him of the sheet tin.

By the present invention the commercial value of tin scrap is materially raised, since it may be utilized for greatly improving and at the same time reducing the cost of manufacture 55 of a high grade article for which there is a decided demand, namely, lead sash weights.

The composite sash weight of the present invention has an exterior surface possessing 60 all the desirable qualities of an all-lead sash weight, but is of a better nature because of the presence of tin scrap in greater or less quantity. Furthermore, the composite sash weight of the present invention is more 65 rigid and less liable to distorting forces than

an all-lead sash weight and permits the utilization of a large proportion of a cheap material in its construction, which material actually improves the article. The only feature wherein the sash weight of the present invention might be compared unfavorably 70 with an all-lead sash weight is in the matter of bulk, but the increased bulk necessary to obtain the desired weight is so slight as to be immaterial.

75 While in Fig. 1 the sash weight is shown as though the tin scrap particles were exposed at the surface thereof, this does not actually occur, since even those edges of the pieces of tin scrap which may come to the 80 surface are coated with lead or a mixture of lead and tin, and consequently are not noticeably visible. Since the lead body forms an envelop covering or encapsulating the 85 particles of tin scrap distributed all throughout the lead body the outer surface of the sash weight is to all intents and purposes a lead surface which is smooth and free from all protuberances of any kind liable to be injurious to the usual wood casing or boxing in which the sash weight moves when installed. The composite material of the sash weight is particularly 90 strong even though it may be in part made of so soft and easily distorted a metal as 95 lead. This great inherent strength is due to the reinforcement provided by the multitude of steel pieces or particles extending in all directions throughout the body of the sash weight and in substantially as firm 100 union with the lead portion of the sash weight as though the lead and the steel were a one piece structure.

105 The particles of tin scrap may be, and usually are, round, square, triangular, and many other shapes both regular and irregular, and under some circumstances are long and slim similar to shreds. Some tin scrap as produced in the course of manufacture of sheet tin articles is in size and shape well 110 adapted for use without further treatment, while other pieces of tin scrap are too large for use in the shape in which they are originally produced. In the latter case they may be bent or otherwise changed in shape 115 and reduced in size, so that they may be readily associated together and with molten lead to form sash weights or other suitable articles for which the composition employed in the present invention is adapted.

120 The term tin scrap is intended to cover the remnants of tin produced in the manufacture of sheet tin articles, whether or not the tin coating has been removed.

125 While the present invention is designed primarily for the production of sash weights, the term sash weight as used herein is designed to include other articles to which the characteristics of the composition or mixture employed are adaptable.

In the foregoing description it has been considered that the sash weight is molded or otherwise formed of lead and tin scrap in practically one homogeneous piece. The 5 sash weight may be formed of a series of blocks or washers of composite material consisting of lead and tin scrap, said blocks or washers being formed in any suitable manner as by punching the blocks or washers out 10 of a sheet of the composition, or in the case of the blocks being each of considerable length, but less than the completed sash weight, they may be molded as hereinbefore described. 15 Such a composite sash weight is illustrated in Fig. 4. The lead and tin scrap composition is formed into blocks or washers 10 each having an axial passage 11 therethrough, and these blocks are strung upon a sustaining rod 12 having an eye 13 at one end and a terminal threaded portion 14 at the other end to which there is applied a nut 15 and an interposed washer 16.

The blocks 10 may have any desired contour, that is, they may be of cylindrical shape or polygonal in cross-section or, in fact, may be any shape desired.

It is desirable that sash weights shall agree as nearly as possible with the weight of the 25 sash they are to balance, and as sashes vary greatly in weight it is usually necessary to obtain sash weights by order, and dealers do not usually carry the sash weights in stock.

With a structure such as illustrated in Fig. 35 4 it is quite feasible to carry in stock an ample supply of blocks 10 of various sizes and shapes and also to carry in stock a supply of rods 11. In the event of an order for sash weights of some certain weight they 40 may be furnished in very close conformity to the weights of the sash by a selection of blocks 10 of such sizes that their combined

weight when strung upon a rod 11 and secured thereon will be practically that of the sash they are to balance.

45

What is claimed is:—

1. A sash weight comprising a mixture of particles or pieces of tin plate and lead with the latter in tenacious adherence to the basic metal of the tin plate and the particles or 50 pieces of the tin plate distributed throughout the article.

2. A sash weight comprising an intimate mixture of tin plate scraps and lead with the latter in tenacious adherence to the basic 55 metal of the tin plate scraps, and said tin plate scraps being in predominant quantity and distributed throughout the lead.

3. A sash weight composed of lead and pieces or particles of tin plate scrap with said 60 pieces or particles distributed throughout the lead and said lead and tin scrap united while the lead is in the molten condition.

4. A sash weight composed of a mixture of lead and pieces or particles of tin plate 65 scrap distributed throughout the lead with the tin coating of the tin scrap alloyed with the lead and the basic metal of the tin scrap tenaciously united to the alloy.

5. A sash weight, comprising a body of 70 lead with tin plate scraps distributed therethrough with the original tin coating of the tin scraps replaced by an alloy of lead and tin having the lead greatly predominating, and said alloy being tenaciously adherent to 75 the basic metal of said tin plate scraps.

In testimony that I claim the foregoing as my own, I have hereto affixed my signature in the presence of two witnesses.

WALTER J. PHELPS.

Witnesses:

JOHN H. SIGGERS,  
JOHN R. RAY.

Copies of this patent may be obtained for five cents each, by addressing the "Commissioner of Patents, Washington, D. C."